

Feb. 14, 1956

E. MARBURG

2,734,242

INGOT MOLDS

Filed June 30, 1954

4 Sheets-Sheet 1

FIG. 1.



Inventor:  
EDGAR MARBURG,  
by: Donald G. Dalton  
his Attorney.

Feb. 14, 1956

E. MARBURG

2,734,242

INGOT MOLDS

Filed June 30, 1954

4 Sheets-Sheet 2

FIG. 2.



Inventor:  
EDGAR MARBURG,  
by: Ronald G. Dalton  
his Attorney.

Feb. 14, 1956

E. MARBURG

2,734,242

INGOT MOLDS

Filed June 30, 1954

4 Sheets-Sheet 3

FIG.3.



FIG.4.



FIG.8.



FIG.5.



FIG.6.



FIG.7.



FIG.9.



FIG.10.



Inventor:  
EDGAR MARBURG,

by Donald G. Dalton  
his Attorney

Feb. 14, 1956

E. MARBURG

2,734,242

INGOT MOLDS

Filed June 30, 1954

4 Sheets-Sheet 4

FIG.11.

TEMPERATURES MEASURED  $\frac{1}{4}$  INCH FROM INSIDE AND OUTSIDE SURFACES  
AND AT MID-THICKNESS.



FIGURES ON CURVES DENOTE  
MINUTES AFTER POUR.

LEGEND

- MOLD OF FIG. 8.  
- - - CONVENTIONAL MOLD WITH WALLS  
OF UNIFORM TAPER.  
OVERALL HEIGHT OF MOLD 26 IN.  
HOT TOP SET 1 INCH  
BELOW TOP OF MOLD.

Inventor:  
EDGAR MARBURG,  
by: Donald G. Dalton  
his Attorney.

1

2,734,242

## INGOT MOLDS

Edgar Marburg, Pittsburgh, Pa., assignor to United States Steel Corporation, a corporation of New Jersey

Application June 30, 1954, Serial No. 440,353

4 Claims. (Cl. 22—139)

This invention relates to improvements in ingot molds. The present application is a continuation-in-part of my earlier copending application Serial No. 299,635, filed July 18, 1952, now abandoned.

Both the uniformity of composition and the internal soundness of a steel ingot are dependent upon its mode of solidification. In changing from the liquid to the solid state, steel contracts about 4 percent; in cooling from the solidus temperature (at which solidification is just complete) to atmospheric temperature, steel contracts an additional 7 percent. As a result of contraction during solidification and cooling, a central cavity or pipe, which may extend below mid-height, develops in ingots cast without top protection. The continuity of the pipe may be broken by bridging; that is, complete trans-solidification, at one or several places below the top of the ingot. Pipe cavity above the uppermost bridge is called open or primary pipe; that below this bridge is referred to as secondary pipe. To prevent pipe from developing in ingots, collars of refractory insulating material (generally fire-clay) are set on mold tops; they extend a few inches down inside the mold. The hot top is poured after the mold is filled. Since the metal in the hot top, or sinkhead, remains liquid longer than that in the ingot body, it may drain into the latter and compensate for ingot shrinkage. For the purpose of describing and claiming the present invention, I define the term "ingot body" as referring to the portion of an ingot below the hot-top junction (plane of lower edge of hot top) in a hot-topped ingot, and the entire ingot below the height of pour in a non-hot-topped ingot.

Initial solidification of ingots occurs approximately according to Feild's Equation  $d=k\sqrt{t}$  ( $d$ =depth in inches;  $t$ =time in minutes). If  $d$  be plotted against  $t$  in this equation, a parabolic curve results. According to this curve, rates of solidification are extremely fast near the surface of an ingot body; they decrease to slow rates in the interior.

Steel solidifies as dendrites, or tree-like crystals. Since purer metal solidifies at a higher temperature than that at which less pure metal solidifies, the solidifying crystals are always purer than the adjacent liquid metal. In particular the layer of liquid metal immediately adjacent to the face of solidification has a higher content of segregating elements, principally carbon, phosphorus and sulphur, than does either the solid metal or the remaining liquid metal. The degree of segregation that occurs is a function of the rate of heat extraction. Near the surface of an ingot body, where heat extraction and solidification rates are extremely fast, little or no segregation occurs; as solidification rates decrease inwardly, the intensity of segregation in the segregated layer increases.

The segregated liquid layer may be entrapped by the following mechanism: elongated or columnar crystals grow inwardly approximately perpendicular to the surface of an ingot body. A columnar dendrite may grow slightly in advance of its neighbors, and penetrate the segregated liquid layer. Since the segregated layer is slightly in-

2

sulating, penetrating columnar crystals provide a preferred course for heat flow. Thus solidification may proceed inwardly and upwardly beyond the segregated layer, and entrap the latter. Because transverse solidification proceeds inwardly at the same time, the above mechanism results in layers of segregation that slope inwardly toward the top of the ingot body, known as inverted-V segregation. In large ingots the above mechanism is repeated, and a series of approximately parallel lines of inverted-V segregation is developed.

Another type of segregation in ingots is V segregation, which occurs along the vertical axis. V segregation results from the entrapment of segregated liquid layers adjacent to the face of vertical solidification by the solidification at higher temperature of purer metal above the segregated layers. V segregation is most concentrated in the upper portions of ingot bodies and decreases in intensity downwardly. In big-end-up ingots V segregation is generally confined to the upper 15 percent of the ingot body; it may extend below mid-height in big-end-down ingots.

If liquid metal be completely entrapped by solid metal, pores or voids result from contraction of the entrapped metal in solidifying. Thus porosity of a minor degree is associated with both V and inverted-V segregation. Major porosity develops along the vertical axes of ingots of certain steels as a result of the entrapment of a vertical column of incompletely solidified metal by trans-solidification just below the hot-top junction. This defect, referred to as axial porosity, is somewhat similar in appearance to V segregation. But, whereas the latter is primarily segregation with associated porosity, the former is V porosity with associated segregation.

The axial defects described above, V segregation and V porosity, are the most serious internal defects in ingot bodies, and are objectionable for many product applications. Because of high breakage in forming sheet and strip products from the upper portions of ingot bodies, the top cuts of ingot bodies of deep-drawing steels are often diverted to other use. Forging may cause internal cracks to develop in ingot bodies with unsound centers; axial defects may also cause weakness in forged products or adversely affect their surface appearance. In products that are center-drilled or bored, center segregation may adversely affect tool life, and/or may cause defects in surface of bore. Laminations in sheet or strip product, blisters in galvanized sheet or strip product, and pinholes in tin plate are other product defects caused by unsound ingot centers.

An object of the present invention is to provide improved ingot molds which minimize axial segregation and porosity in ingot bodies cast therein.

As hereinafter explained, it is desirable that ingot bodies solidify as rapidly as possible in a vertical direction upwardly from the bottom, and as slowly as possible transversely across the top; a further object is to provide ingot molds which promote vertical solidification, and retard transverse solidification across the top.

A further object is to provide ingot molds in which the foregoing objects are attained by simple proportioning of the thickness of various parts of the mold walls.

In accomplishing these and other objects of the invention, I have provided improved details of structure, preferred forms of which are shown in the accompanying drawings, in which:

Figure 1 is a schematic view which shows a typical solidification pattern of a big-end-up ingot;

Figure 2 is a schematic view which shows a typical solidification pattern of a big-end-down ingot;

Figure 3 is a top plan view of a big-end-up ingot mold which embodies features of the present invention;

Figure 4 is a side elevational view of the mold shown in Figure 3, the mold being equipped with a hot top;

Figure 5 is a horizontal sectional view taken on line V—V of Figure 4;

Figure 6 is a horizontal sectional view taken on line VI—VI of Figure 4;

Figure 7 is a horizontal sectional view taken on line VII—VII of Figure 4;

Figure 8 is a vertical sectional view of a big-end-down mold constructed in accordance with the invention, the mold being equipped with a hot top;

Figure 9 is a view similar to Figure 8, except that the mold lacks a hot top;

Figure 10 is a vertical sectional view of a modified form of a big-end-down mold in accordance with my invention, the mold being equipped with a hot top; and

Figure 11 is a graph which compares mold wall temperatures of a mold constructed as shown in Figure 8 with those of a conventional mold.

The progress of solidification of an ingot body may be depicted by isochrones representing the face of solidification at various intervals after pour. Figure 1 shows the solidification pattern of a 32 by 32 inch big-end-up ingot reconstructed from measurements of shell thicknesses of six ingots dumped at various intervals after pour. Figure 2 shows a solidification pattern for the 29-inch-wide section of a 29 by 66 inch big-end-down ingot. Although the patterns for the big-end-down and the big-end-up ingot are generally similar, they differ in certain important respects, to be discussed below. The patterns may be considered from three viewpoints: (a) solidification transversely from sides to middle; (b) solidification vertically from base to top; and (c) accelerated solidification resulting from overlapping of transverse and vertical components of heat extraction, originating at points of tangency *a*, Figure 1, between straight sides and curved base of a big-end-up ingot, or at the corners, *a*, Figure 2, of a square-based big-end-down ingot.

Lines *af* represent loci of acceleration of transverse solidification originating at critical points *a*. Outside the lines *af* the face of transverse solidification proceeds parallel to the sides of the ingot approximately according to Feild's Equation  $d=k\sqrt{t}$ . I have found that inner lines of inverted-V segregation develop as a result of acceleration of transverse solidification; hence they coincide with loci *af* of this acceleration. Accelerated transverse solidification is first completed to the middle of the ingot at point *c*, which represents the tip of the base cone *abaca* of vertical solidification. When trans-solidification is completed at *c*, there remains a relatively large column of liquid metal above point *c*, as bounded in Figure 1 approximately by isochrone 100. At point *c* transverse components of heat extraction from all four sides of the ingot are added to vertical components effecting vertical solidification. As a result, vertical solidification rates are greatly accelerated at point *c*, as indicated by the wide spacing of isochrones along the vertical axis above this point. Because of the extremely fast rates of final accelerated vertical solidification above point *c*, vertical solidification reaches the top of the ingot body before transverse solidification is completed across the top. Dashed lines *ec* trace the cores of vertical solidification thus developed in ingot bodies of both types.

I have found that V segregation is developed within and extends across the vertical cores of ingot bodies. Since segregates are lighter than liquid steel, they have a tendency to float upwardly and escape into the sinkhead. Their ability to do so, however, depends upon the width of the vertical core and that of the adjacent zones of accelerated transverse solidification at the hot-top junction, that is, upon widths  $V_t$  and  $V_a$ . As indicated by the solidification patterns,  $V_t$  and  $V_a$  are wider in big-end-up ingots than in big-end-down ingots of comparable sizes. For this reason, the former ingot bodies develop less axial segregation and porosity than do the latter.

Widths  $V_t$  and  $V_a$  are principally dependent upon two factors; (1) the width to height ( $w/h$ ) ratio of an ingot body, and (2) the ratio of the rates of transverse solidification across the top of the ingot body to those of vertical solidification. Wide vertical cores and sound ingot bodies are favored by high  $w/h$  ratios. Practical limitations of rolling mill equipment and economic considerations, however, dictate the upper limit of  $w/h$  ratios of ingot bodies. It would almost certainly prove uneconomical to increase  $w/h$  ratios of ingot bodies to the extent necessary to eliminate all axial defects.

Wide vertical cores (and sound ingot bodies) are also favored by slow rates of transverse solidification across the top of an ingot relative to vertical solidification. Since experiments have demonstrated that transverse solidification rates vary with mold-wall thickness (at least in mold walls over 2 inches thick), it would naturally seem desirable to design mold walls thin at the top, and thick at the base (since rates of accelerated vertical solidification in the vertical core are caused principally by transverse components of heat extraction to the lower portion of the mold wall). Indeed, mold walls are commonly so designed, with the base 1 to 4 inches thicker than the top, and with a uniform taper between the two ends. Unfortunately, however, tapered mold walls are ineffective in producing differential solidification in ingots. Numerous dumped-ingot experiments have revealed that, except for accelerated solidification from the base, solidification proceeds at uniform rates throughout the height of ingots cast in molds with tapered walls. It is extremely difficult to analyze exactly heat losses from mold walls. Heat will flow through the walls, vertically as well as transversely, from hotter to colder portions. In addition to conducted heat, heat will be radiated from the outer surface in amounts varying with the surface temperature. Regardless of the exact analysis of heat losses from mold walls, however, it is well-known that molds become hotter in their middle portions than at their end portions (this can be verified by observation; an oval-shaped portion in the middle of each wall becomes heated to a bright red to orange color, while the end portions remain dull red to black). Since heat-extraction rates will vary inversely with mold temperatures, however, it is undesirable to have a higher temperature at the middle than at the top of the mold wall.

The purpose of the present mold design, as will be clear from the following description, is to control temperatures in mold walls so as to cause greater rates of transverse heat-extraction from the base and middle than from the top portion of a mold, hence to cause solidification to proceed in a favorable manner.

Figures 3 to 7 show a big-end-up mold constructed in accordance with my invention. This mold is equipped with a hot top *H* which is of any standard or desired construction and extends a short distance into the top of the mold cavity. The upper portions 10 of the mold walls are thin and the lower portions 12 thick. Immediately below the bottom of the thin upper portion 10 is a relatively short, thickened section 13. Between this thickened section and the top of the thick bottom portion 12 is a relatively short thin section 14. The trace of the inside surface of the walls in any vertical plane above the base is a straight line.

When molten steel is introduced to the mold just described, the thin portions 10 and 14 become hotter than the thick portions 12 and 13. Consequently heat flows from the top portion 10 and from the thin section 14 into the thick section 13, as indicated by arrows. Hence a horizontal plane may be passed through section 13 across which no vertical heat flow occurs. Similarly heat flows upwardly from thin section 14 into thick section 13 and downwardly from thin section 14 to thick portion 12. Hence a horizontal plane across which no vertical heat flow occurs may also be passed through thin section 14.

Because of the middle thick-and-thin arrangement, heat

from the upper thin portion 10 flows downwardly into the comparatively small volume represented by the upper half of the thick section 13. Similarly the lower thick portion 12 receives heat only from the lower half of thin section 14. Thus the normally faster rates of solidification of thick base portion 12 and normally slower rates of thin upper portion 10 are disturbed to a minimum extent. As a result, the thin top and thick base portions of molds are enabled to effect differential solidification in ingots in the manner desired.

Figure 8 shows a big-end-down mold constructed in accordance with my invention. This mold is equipped with a hot top H similar to that shown in Figure 4. The mold walls have a relatively thick lower portion 17 and a relatively thin upper portion 18. At the bottom of the latter is a relatively narrow thick section 19. Between the thick section 19 and the top of the thick lower portion 17 is a relatively narrow thin section 20. The trace of the inside surface in any vertical plane again is a straight line. Thick section 19 and thin section 20 act to disrupt vertical flow of heat in the same manner as the corresponding thick section 13 and thin section 14 in the big-end-up mold shown in Figures 3 to 7.

Figure 9 shows a big-end-down mold which is similar to Figure 8, except that it lacks a hot top. Semi-killed, or gas-evolving steels, such as represented in Figure 2, are commonly cast without hot tops. Molten metal is poured into the mold to a height a few inches short of the mold top. The height of ingot body cast therein is comparable to the portion of a hot-topped ingot below the hot-top junction. The solidification pattern of this ingot, Figure 2, has already been discussed.

Figure 10 shows an alternative mold construction which can be used to facilitate manufacture. Although Figure 10 shows a big-end-down mold equipped with a hot top, it is apparent that the same mold can be used without a hot top and that the same principles can be applied to a big-end-up mold. In large foundries, a sand slinger frequently is used to make the outer sand mold for casting the ingot mold. A sand slinger has revolving blades which throw sand with tremendous force into the peripheral space between an outer housing and the pattern (similar to the ingot mold exterior). It is apparent that sand so placed would not pack tightly in the "dead space" below the thick ring 13 of Figure 4 or 19 of Figures 8 and 9. Consequently the mold shown in Figure 10 has a thickened portion 22 and a thinner portion 23 separated by a re-entrant angle modified to enable sand to be packed tightly with a slinger. The action of the thick and thin portions in the mold walls is the same as already described for the other embodiments.

Height  $d$  in Figures 4, 8, 9 and 10 represents the vertical distance between the top of the ingot body and the beginning of the uppermost thickened section and may be evaluated as about 10 to 70 percent of the height of the ingot body. While these are extreme limits of effectiveness, the preferred range is about 35 to 50 percent of the height of the body. The actual mold extends a few inches above this height to allow for insertion of a hot top or to leave some clearance above the height of pour in a non-hot-topped ingot. The minimum spacing  $c$  can be as low as it is practicable to cast corrugations. The upper limit of spacing may be specified as about 24 inches. While these are extreme limitations, the preferred spacing of corrugations is about 12 inches.

Figure 11 shows a graph which demonstrates the effectiveness of my invention. In this graph the solid line curves represent mold wall temperatures at various vertical positions and at various intervals after pour with a mold constructed as shown in Figure 8, of inside dimensions  $7\frac{1}{2}$  by  $7\frac{1}{2}$  inches at the top,  $8\frac{1}{2}$  by  $8\frac{1}{2}$  inches at the base. The broken line curves represent corresponding temperatures in a conventional mold (i. e. a mold whose walls taper uniformly), of the same internal dimensions, and of the same wall thickness at the top ( $1\frac{1}{2}$

inches), and at the base ( $3\frac{1}{2}$  inches) as the mold shown in Figure 8. In each instance the temperatures were determined by inserting a thermocouple in one of the mold walls at the height indicated and to a depth  $\frac{1}{4}$  inch from the inside face, a second thermocouple in another wall at the same height to the mid-thickness depth, and a third thermocouple in a different wall at this height to a depth  $\frac{1}{4}$  inch from the outside face, and averaging the three readings. The broken-line curves show that the conventional mold is hottest at the middle portion; also it is hotter at the base portion than at the top (at least for the time, about 7 minutes, required for most of this ingot to solidify). In an exact opposite manner, the experimental mold is least hot at the middle thick ring for the duration of solidification; it is also less hot at the base than at the top portion. Thus the experimental mold extracts heat faster from the base and middle portion, than it does from the top of an ingot (in the manner desired for favorable solidification).

Another test was conducted in which ingots of 0.25 percent carbon steel cast in the above two molds were back-poured with steel containing 2 percent copper about 6 minutes and 30 seconds after pour. Since steel containing copper etches darker than steel without copper, the metal that had been liquid at back-pour was revealed as a dark column in the macroetch of a longitudinal section of each ingot. Measurements of these macroetches reveal that, at the time of back-pour, transverse solidification had proceeded  $2\frac{1}{4}$  inches across the top of the ingot cast in the regular mold, but only 2 inches across the top of the ingot cast in the mold of special design, Figure 8. Vertical solidification had progressed to a height only about  $5\frac{1}{2}$  inches above the base of the former mold; it had attained a height of 13 inches in the latter mold. These macroetches provide evidence that vertical solidification had progressed almost  $2\frac{1}{2}$  times as far in the mold of special design as in the regular mold; but transverse solidification had only proceeded 86 percent as far across the top of the former ingot.

Ingots of various grades, plain-carbon, low-alloy, and sulfur steels, have been cast in big-end-up and big-end-down molds of the design shown in Figures 4 and 8. Comparison ingots of the same steels have been cast in conventional molds of the same internal dimensions, but of uniform wall taper. The ingots have been split longitudinally along the center plane, machined and ground to a smooth surface, and macroetched. All of the ingots cast in molds of conventional design contained secondary pipe, V segregation and axial porosity to a greater or less extent. In contrast, all the ingots cast in the special molds with one exception (the big-end-down low-alloy steel ingot had some axial porosity) were completely solid and sound.

From the foregoing description it is seen that the present invention affords an effective means for disrupting the vertical flow of heat in ingot mold walls by simple proportioning of the wall thickness. The invention effectively eliminates the most serious axial defects in ingots, namely secondary pipe, V segregation and axial porosity.

While several embodiments of my invention have been shown and described, it will be apparent that other adaptations and modifications may be made without departing from the scope of the following claims.

I claim:

1. An ingot mold comprising solid side walls which define a cavity adapted to receive molten metal for casting an ingot body and which extend a relatively short distance above the normal height of the ingot body, said walls below this height being of greater thickness in their lower portion than in their upper portion to accelerate solidification of the lower portion of an ingot body both transversely and vertically and to retard transverse solidification of the upper portion, the trace of the inside surfaces of said walls in any vertical plane away from the lower end being a straight line, and means on the exterior of said

walls between their thick and thin portions spaced below the normal height of an ingot body by a distance which is 10 to 70 percent of the height of the ingot body for disrupting vertical heat flow in these walls, said means including a thickened section and a thinner section immediately therebelow, both of said sections being of relatively short vertical dimensions.

2. An ingot mold comprising solid side walls which define a cavity adapted to receive molten metal for casting an ingot body and which extend a relatively short distance above the normal height of the ingot body, said walls below this height being of greater thickness in their lower portion than in their upper portion to accelerate solidification of the lower portion of an ingot body both transversely and vertically and to retard transverse solidification of the upper portion, the trace of the inside surfaces of said walls in any vertical plane away from the lower end being a straight line, a relatively short thick section in said walls at the bottom of their upper thin portion spaced below the normal height of an ingot body by a distance which is about 35 to 50 percent of the height of the ingot body, and a relatively short thin section in said walls immediately below said thick section, said thick and thin

sections cooperating to disrupt vertical heat flow in said walls.

3. A mold as defined in claim 2 which is of the big-end-up type and in which the portion of the walls above the normal height of the ingot body is adapted to receive a hot top.

4. A mold as defined in claim 2 which is of the big-end-down type and in which the portion of the walls above the normal height of the ingot body is adapted to receive a hot top when a hot-topped ingot is cast therein and to provide clearance above the height of pour when a non-hot-topped ingot is cast therein.

15 References Cited in the file of this patent

UNITED STATES PATENTS

2,023,833 Gathmann ----- Dec. 10, 1935  
2,626,436 Marburg ----- Jan. 27, 1953

20 FOREIGN PATENTS

16,709 Great Britain ----- of 1908  
530,675 France ----- Oct. 7, 1921